

K. FARKAS.

## PROCESS OF MAKING METALLIC FILAMENTS.

APPLICATION FILED DEC. 13, 1910.

1,188,057.

Patented June 20, 1916.



Fig: 1



Fig: 2

Witnesses:  
Max P. A. Doring.  
Corinne Myers.

Inventor  
Karl Furkas  
By his Attorney L. K. Johnson

# UNITED STATES PATENT OFFICE.

KARL FARKAS, OF GLEN RIDGE, NEW JERSEY, ASSIGNOR TO J. EMIL WALSHEID, OF WEEHAWKEN, NEW JERSEY.

## PROCESS OF MAKING METALLIC FILAMENTS.

1,188,057.

Specification of Letters Patent. Patented June 20, 1916.

Application filed December 13, 1910. Serial No. 597,140.

*To all whom it may concern:*

Be it known that I, KARL FARKAS, a citizen of the Kingdom of Hungary, and a resident of Glen Ridge, county of Essex, and

5 State of New Jersey, have invented certain new and useful Improvements in the Process of Making Metallic Filaments, of which the following is a specification.

This invention has reference to flexible 10 metallic filaments and the process of producing same.

Metallic filaments are usually produced by mixing refractory oxids such as for instance tungsten oxid with glutinous car-

15 bonaceous material that acts as a binder. The carefully prepared uniform mass is then pressed through a die by exceedingly high pressure, in some instances hydraulic pressure is used and a filament heated by

20 the electric current in an evacuated chamber in the presence of hydrogen. This process as generally outlined above, produces metallic filaments that are brittle and very delicate. They are so fragile that they have

25 to be handled with the greatest of care during the manufacture of the lamp and may be broken like fine steel wires. The cause of this extreme fragility of metallic filaments is that it is very difficult to produce

30 filaments which are free from impurities. Traces of foreign metallic oxids or metals or carbonaceous matter and probably carbids formed by the carbon and metal may be found therein and the result is, as above

35 stated a very delicate and fragile filament which is brittle and cannot be bent except after pressing when the glutinous binder is still therein. The filament which has been reduced by hydrogen and is then in the

40 so-called metallic state of course softens when electrically heated while in an exhausted glass receiver or in a finished lamp but this property of the filament at that condition cannot be utilized for shaping filaments for practical purposes.

It is the object of the present invention to produce metallic filaments which are flexible before they are inserted into a lamp when they are already in the metallic state 50 so that same may be shaped into a desired form to such an extent that other than the present shapes of filaments may be made

therefrom. It is self-evident that with such metallic filaments a great saving is effected because the breakage during the manufacture of lamps is reduced to a minimum. 55

In carrying the present invention into effect the refractory oxids are first purified by transforming them into the highest stage of oxidation and after these have been 60 carefully prepared the plastic mass is formed, the filament pressed and the pressed filament is treated in an electric oven wherein it is reduced. This oven is represented in the accompanying drawing in 65

which:

Figure 1 represents in elevation an apparatus for pressing metallic filaments and an electric oven in which they are reduced. Fig. 2 represents in vertical section the electric oven which embodies in desirable form 70 the present improvements.

Similar characters of reference denote like parts in all the figures.

As above stated the refractory oxids, for 75 instance tungsten oxids are first purified by transforming them into the highest state of oxidation. This is accomplished by heating them in an atmosphere of oxygen for the purpose of producing the highest 80 oxids and burning out impurities. By this process oxids are obtained in as pure a condition as possible. The tungstic oxids are, for instance, transformed into tungsten trioxid  $WO_3$  which is yellow and if for the 85 purpose of purification the hydrate was formed for instance  $WO_4H_2$ , the treatment with oxygen serves a further purification. In the described purified tungstic oxids none of the brown tungstous oxids are found any 90 more. The purified tungstic oxids are now reduced to very fine powder and passed through silk sieves so as to separate out only the very finest impalpable powder. This very fine impalpable powder is now 95 passed through tight rollers of the kind of the color rollers until it assumes a metallic luster whereby a very compact powder is obtained. The powder having the metallic luster is now mixed with a pure glutinous and carbonaceous binder. Any of the well approved binders may be used. In preparing the plastic mass about 100 gr. of the impalpable powder of the oxid is mixed 100

with about 2 gr. of the binder. When a homogeneous mass has been obtained same is placed into the filament press *a*, shown in Fig. 1, from which the filament *b* issues and passes into the electric oven *c*. The filaments are pressed very slowly so that at the best ten inches of filament are produced per minute.

The electric oven through which the filament passes is shown in section, in Fig. 2. The oven consists of an inner porcelain tube *d* shown in elevation. Around this porcelain tube nickel wire *e* is wound at such distance that it is insulated by the porcelain of which the tube is composed. In this way this inner porcelain tube *d* may be electrically heated. This tube is open. A second porcelain tube *t* surrounds the tube *d*. This tube is closed at the top and bottom except to note that a pipe *f* leads into same for the purpose of introducing a gas into same. The second porcelain tube is surrounded by nickel wire *g* or the like so that same may be electrically heated. Both tubes are enclosed into a steel shell *h* and the space between the layer of wire *g* and the walls of the steel or iron shell is filled with asbestos *i*. The surrounding shell *h* is so constructed that it closes the porcelain tube *t* but leaves the tube *d* open. Centrally at the top of the shell *h* there is a conducting roller *j* and at the bottom a like roller *k* on which the filament *b* is conducted through the oven and by means of these conducting rollers *j* and *k* the filament may be electrically heated while it passes through the oven.

When starting to make filaments hydrogen gas is continuously passed through the inner porcelain tube *d* from below whereby first of all the air is expelled. The space within the porcelain tube *t* is also filled with hydrogen gas through the tube *f* and sufficient gas is passed through to expel the air. When this has been done the hydrogen within the tube *t* is constantly kept therein and not renewed. Now the porcelain tubes are electrically heated and the filament likewise is electrically heated in the atmosphere of hydrogen which constantly passes through the tube *d*. By heating the porcelain tubes electrically the hydrogen of course gets very hot and in this condition has great reductive power. The filament entering the electric oven consists of the plastic material formed out of the refractory pure oxids and a pure organic binder. When entering the porcelain tube *d* the filament is reduced by the heated hydrogen and after passing the lower conductive roller *k* the filament itself is electrically heated whereby a complete reduction to pure metal takes place. By the heated hydrogen and by heating the filament electrically all oxids are reduced and all organic matter from the binder is completely burned out. Simultaneously the in-

closed hydrogen atmosphere in the tube *t* is heated by the hot porcelain tubes and thus aids in the production of a terrific heat within the electric oven. The filament when leaving the roller *k* is now wound on suitable rolls and is flexible like metallic wire and may be formed into various shapes of filaments. In fact it is pure metallic wire after the treatment in the electric oven and may be handled as such and drawn out into still finer wire if desired.

I claim as my invention:

1. The process of producing flexible metallic filaments for incandescent electric lamps consisting in passing successively and continuously each portion of the pressed filament, while said portion is rendered incandescent, through a continuously flowing current of heated hydrogen surrounded by a heated stationary atmosphere of hydrogen, whereby the filament is reduced to a pure metallic state.

2. The process of producing flexible tungsten filaments for metallic filament lamps consisting in passing successively and continuously each portion of the pressed filament, while said portion is rendered incandescent, through a continuously flowing current of heated hydrogen surrounded by a heated stationary atmosphere of hydrogen, whereby the filament is reduced to a pure metallic state.

3. The process of producing flexible metallic filaments for incandescent electric lamps consisting in pressing continuously a filamentary thread and passing successively and continuously each portion of the pressed filament, while said portion is rendered incandescent, through a continuously flowing current of heated hydrogen surrounded by a heated stationary atmosphere of hydrogen, whereby the filament is reduced to a pure metallic state.

4. The process of producing flexible tungsten filaments for metallic filament lamps consisting in pressing continuously a filamentary thread and passing said thread directly, portion by portion, while each portion is rendered incandescent, through a continuously flowing current of heated hydrogen surrounded by a heated stationary atmosphere of hydrogen, whereby the filamentary thread is reduced to a pure metallic state, and then shaping filaments therefrom.

5. The process of producing flexible metallic filaments for incandescent electric lamps consisting in passing successively each portion of the pressed filament composed of highly refractory oxids while being rendered incandescent through a continuously flowing current of heated hydrogen surrounded by a heated stationary atmosphere of hydrogen, and reducing the filament thereby.

6. The process of producing flexible tung-

sten filaments for metallic filament lamps consisting in passing successively each portion of the pressed filament through a continuously flowing current of heated hydrogen, while being rendered incandescent therein, said current of heated hydrogen being surrounded by a heated stationary atmosphere of hydrogen reducing the filament thereby to pure tungsten wire which is flexible before being placed in the lamp. 10  
Signed at New York, N. Y., this 12th day of December, 1910.

KARL FARKAS.

Witnesses:

CORINNE MYERS,  
VERA PAULSEN.

Copies of this patent may be obtained for five cents each, by addressing the "Commissioner of Patents, Washington, D. C."